

# UNITED STATES PATENT OFFICE.

LINDON WALLACE BATES, OF MOUNT LEBANON, NEW YORK.

## FUEL AND METHOD OF PRODUCING SAME.

1,375,811.

Specification of Letters Patent. Patented Apr. 26, 1921.

No Drawing. Original application filed August 5, 1919, Serial No. 315,497. Divided and this application filed January 22, 1920. Serial No. 353,324.

To all whom it may concern:

Be it known that I, LINDON W. BATES, a citizen of the United States, residing at Mount Lebanon, in the county of Columbia 5 and State of New York, have invented certain new and useful Improvements in Fuel and Methods of Producing Same, of which the following is a specification.

This invention pertains to a stable mobile 10 fuel containing liquid hydrocarbon whose asphaltic and free carbon particles are stabilized. It is well known that crude and refined oils, such as oils from Mexico and pressure still oil or tar contain asphaltic 15 particles and also particles of free carbon which tend to settle and limit seriously the utility. In my copending application Serial No. 315,497, filed August 5, 1919, the stabilizing qualities of lime-rosin soap, the pep- 20 tizing and stabilizing qualities of certain derivatives of coals, or their equivalents, were fully described. The quantity of from about  $\frac{1}{2}\%$  to 2% of a resinous soap with alkali will stabilize for a considerable period 25 up to several months carbonaceous particles up to 40% by weight incorporated into a liquid fuel. Adequate stability or non-separa- 30 tion of the components for a reasonable time and to a suitable degree to allow prac- tical use of the fuel may also be obtained by 35 percentages from about 1% to 10% of coal distillate such as creosote or naphthalene or solvent naphtha tar. Furthermore, about 20% of coal tar will stabilize 30% coal par- 40 ticles in some oils. These various classes of stabilizing substances are not all equally effective but all produce adequate fuel sta- 45 bility for a desired period of reasonable length and may be combined in use.

It is possible, furthermore, as stated, to 50 obtain over a year's stability of the asphaltum and free carbon particles encountered as natural impurities in pressure still oil by the use of such amount of lime-rosin grease 55 as will add 1% rosin into the oil. This applies to other liquids also. Distillates of coal and other carbonaceous substance act to peptize and so stabilize not only particles of solid carbonaceous substance introduced 60 into such oils or tars but also the natural carbonaceous impurities, such as asphaltum and free carbons encountered therein.

The method of combining the stabilizing substance or substances with the liquid con- 65 sists in a mechanical or heat treatment or

both. The mechanical treatment may consist in agitating the components together in a mill, such as a coal pulverizing or other blending mill. Heat may be applied or occur in the mill or elsewhere in a suitable vessel. The requisite heat varies and may attain 95° C. or over, depending on whether heat alone is relied upon or mechanical blending is added. So also the combined treatment may be briefer than may the latter 65 alone. By the addition of any or several of the substances stated, the natural carbonaceous impurities in the liquid hydrocarbons may be so treated as to produce a stable fuel. If a plurality of such substances 70 is used the amount of each may be less than the percentages indicated. So also buoyant substance may be added to the liquid to delay settling, and viscosity may be adjusted if for any reason it is convenient. Gener- 75 ally speaking, the method and procedure, outlined in my said copending application apply fully to this application of which this is a division.

It should of course be emphasized that the 80 lime-rosin soap or its equivalent should be carefully prepared, as its efficiency depends upon the degree of saponification and the condition of the soap, in a carrier such as oil. The method of making a suitable lime- 85 rosin grease is fully described in my co- pending application. Less carefully prepared resinous soaps will not give the same 90 stability as the well prepared. Considerable research was necessary to produce an ade- 95 quate saponaceous fixture or soapy stabilizing substance. Unless otherwise stated, the addition of larger amounts of stabilizing substances than the percentage necessary to obtain stability does not produce injurious results. This is also the case when fillers or other lighter substances are added to promote stability, or viscosity adjusting liquids or other substances are added to adapt the 100 fuel for any special purpose.

What is claimed is:-

1. That method of stabilizing the asphaltum and free carbon particles in liquid hydrocarbon containing the same, which consists in blending therewith coal distillate or 105 equivalent peptizing substance and blending the components and simultaneously peptizing the particles with heat treatment at a temperature range between normal tempera- 110 ture and approximately 95° C.

2. A stable liquid fuel consisting entirely of liquid hydrocarbon, asphaltum and free carbon particles encountered therein only, and a small amount of lime-rosin grease or 5 equivalent stabilizing substance.

3. A stable liquid fuel consisting entirely of liquid hydrocarbon, asphaltum and free carbon particles encountered therein only,

coal distillate having peptizing qualities upon the particles, and a small amount of 10 lime-rosin grease or equivalent stabilizing substance.

In testimony whereof I have signed my name to this specification.

**LINDON WALLACE BATES.**